

## UNITED STATES PATENT OFFICE

JULIAN L. SCHUELER, OF KOKOMO, INDIANA, ASSIGNOR TO CONTINENTAL STEEL CORPORATION, OF KOKOMO, INDIANA, A CORPORATION OF INDIANA

## ALLOY STEEL

No Drawing.

Application filed November 27, 1931. Serial No. 577,713.

This invention has reference to an alloy steel, the components of which include copper, nickel and chromium in the low percentage ranges.

I am aware that steels have been made, the components of which include copper, nickel and chromium in the high percentage ranges, such as are used for acid resisting steels and where the ultimate cost of producing and 10 where the sales cost is high. This is due to the fact that copper, nickel and chromium are high priced elements, especially the latter two, and their addition to steel in large amounts involves a very high and specialized 15 metallurgical practice in addition to the cost of the materials themselves. Furthermore, if resistance to corrosion is to be a characteristic, using these materials in the high percentage range requires the steels to be heat 20 treated in a proper manner in order to bring out all of their physical properties, including that of resistance to corrosion.

It is an object of my invention to produce an alloy steel from which may be manufactured materials intended especially for farm use, where the cost is a material item and which materials are subjected to and will resist atmospheric corrosion, thereby insuring long life and a maximum of use. The materials I have in mind are farm fencing and the like; sheets for roofing, siding, gutters, ridge roll and the like, for building purposes, and for culvert stock. Any or all of these products may be readily coated with a hot dipped 25 galvanized coating, which can be readily formed and subjected to severe drawing and stamping operations, without the coatings cracking or flaking. Steels including copper, nickel and chromium in the high percentage 30 ranges cannot be employed for the uses herein enumerated because the cost is prohibitive. Furthermore, to employ the steel of my invention for the uses stated requires no heat treatment and they will retain their maximum 35 resistance to corrosion, regardless of this factor.

The necessity for a relatively cheap steel which will resist atmospheric corrosion, is, at the present time, of the utmost importance; 40 but the only cheap steels available for this

purpose, so far as I am aware, are the copper steels containing around .20% copper.

It is a well accepted fact, among those skilled in the art, that ordinary steel containing about .20% of copper will outlast an ordinary carbon steel, when subjected to atmospheric corrosion from one and one-half to three times or more. This has been amply proved by a long series of tests conducted by the American Society for Testing Materials, 50 and no experimental evidence has ever been offered to disprove this fact.

It has also been demonstrated that with steel containing above .20% copper, no added corrosion resistance is obtained, due primarily to the fact that the copper above that percentage does not form a solid solution with the steel, or at least does not unite with the steel in the form to give any added protection. I have discovered, however, that copper, up to double this amount, may be added 70 to the steel and a far better resistance to atmospheric corrosion obtained when nickel and chromium are also present in the steel.

I have found that steels containing from .10% to .40% copper; .75% to .20% nickel and .70% to .07% chromium, will outlast, under a great many corroding conditions, especially atmospheric corroding conditions, steels containing either one or the other of these elements alone, in the percentages stated. For example, the steel containing .10% to .40% copper, or containing .75% to .20% nickel, or a steel containing .70% to .07% chromium, 80 will not resist corrosion as well as a steel containing the three elements as given. For example, I have made copper, nickel, chromium steels of the following analyses:

|            | Per cent |    |
|------------|----------|----|
| Carbon     | .08      | 90 |
| Manganese  | .40      |    |
| Phosphorus | .004     |    |
| Sulphur    | .040     |    |
| Silicon    | .010     | 95 |
| Copper     | .30      |    |
| Nickel     | .50      |    |
| Chromium   | .08      |    |

These are merely cited as examples and not as limiting factors. For example, for 100

killed steel, the silicon, instead of being .01%, might be .14% and so on. Furthermore, for certain physical properties, the carbon may be much higher; as within the copper, nickel, chromium range, which I employ, neither the copper, nickel or chromium interfere with the heat-treating properties of the steel, per se. Furthermore, I have found that heat treating has no marked effect on the corrosion resisting properties of this steel, which is not the case with very high percentage chromium, nickel alloy steels.

It will, of course, be realized that the proportion of copper, nickel and chromium within the limits specified can be subject to any combination. The combinations I have recited are typical and I have found that very good results are obtained when the sum of the copper plus nickel is approximately .70% to .80% with chromium about .30% to .20%; or the sum of the copper plus chromium is approximately .70% to .80% with nickel about .30% to .20%.

I have found that the addition of copper-nickel-chromium to the steel, is materially beneficial and still the high percentage ranges are not necessary as are required in the very high priced alloy steels, such as are used for acid resisting steels. Such an alloy steel as I disclose is more easily made in the open hearth furnace and the homogeneity of the steel is more easily controlled than where large amounts of copper, nickel and chromium would be used separately, or in combination of any two. Furthermore, the addition of these elements imparts superior physical properties in the way of additional tensile strength and toughness, besides the corrosion resisting value, than is the case of any one or any combination of the two, in the proportions herein disclosed. As a consequence, alloy steels such as I describe are excellent for the manufacture of woven wire fence and sheets, particularly where such fencing or sheets are subject to atmospheric exposure. And as pointed out, these steels galvanize very nicely and may be formed in severe drawing operations. Also, they may be welded, either electrically or by gaseous processes, which is not always true of the high percentage alloy steels.

What I claim is:—

1. A corrosion resisting steel alloy containing copper from .10% to .30%, nickel from .30% to .50%, chromium from .07% to .30%, and the balance substantially iron.

2. A corrosion resisting steel alloy consisting of carbon about .08%, manganese about .40%, phosphorus about .004%, sulphur about .040%, silicon about .010%, copper about .30%, nickel about .50% and chromium about .08%.

3. A corrosion resisting steel alloy containing .10% to .30% of copper, about .30%

of nickel, about .07% to .30% of chromium, and the balance being substantially iron.

In witness whereof, I have hereunto set my hand, this 25th day of November, 1931.

JULIAN L. SCHUELER. 70

75

80

85

90

95

100

105

110

115

120

125

130